

## UNITED STATES PATENT OFFICE

LADISLAV RYS, OF RUZOMBEROK, CZECHOSLOVAKIA

## METHOD FOR BLEACHING CELLULOSE OF ANY KIND

No Drawing. Application filed December 20, 1928, Serial No. 327,458, and in Czechoslovakia December 19, 1927.

This invention relates to a method for bleaching cellulose of any kind.

Aqueous solutions of alkali-metal hypochlorites or bleaching powder are the usual bleaching agents for bleaching cellulose. It is known in the art, to subdivide the bleaching process of cellulose with the above described bleaching agents into two separate steps, namely a preliminary bleaching process and an after-bleaching process, between which the pre-bleached cellulose is washed, thus saving chlorine, when comparing this way of proceeding with those methods in which the whole amount of bleaching liquor is added at once to the cellulose to be bleached.

This saving of chlorine is due to the fact that a certain amount of oxidizable substances, liberated by the pre-bleaching process are removed by the intermediate washing process.

It is further known, to improve the bleaching process by using cellulose concentrations of 15 to 24% instead of 5-8% as formerly, thereby increasing the rate of reaction during the bleaching process, avoiding heating of the reaction mixture and reducing the amount of chlorine necessary. The disadvantage of a bleaching process with high cellulose concentration is, however, to be seen in the fact, that the mixing of the viscous cellulose with the bleaching liquor is somewhat troublesome.

It is also known to bleach cellulose, which if necessary has been subjected to a preliminary treatment with alkali metal or alkaline earth metal hydroxides or with alkali metal sulfites or bisulfites, by treatment with chlorine, repeated if necessary, before or after the bleaching process with alkaline peroxides with the addition of alkali metal silicates. It is also known to subject material, which has been first bleached in the usual way, for example, with alkali hypochlorites, to a subsequent bleaching, repeated, if necessary, with chlorine.

However, these processes involve intensive treatment with considerable amounts of chlorine and for this reason injury to the material treated cannot be avoided even though the excess chlorine remaining in the material is removed by subsequent treatment with sodium hyposulfite, for example. Further-

more, the cost of the comparatively large amount of chlorine used in these processes makes them expensive.

I have found that excellent results are obtained if, in the prebleaching with chlorine, the chlorine is used in the gaseous form or as chlorine water only in an amount up to about 90% of the total amount necessary for complete bleaching and if the bleaching is then completed by applying the remainder of the necessary chlorine in the form of hypochlorite. In this manner, the bleaching can be performed with greatest simplicity, with greatest sparing of the fibers of the material treated and with great saving of materials.

I have found further that the amount of chlorine used in the pre-bleaching can be still further substantially limited if the material to be bleached is washed with dilute alkalies such as sodium hydroxide, milk of lime and the like, before the chlorine treatment, whereby at the same time it is possible to avoid coloration of the fiber under the influence of the chlorine, which coloration would require the use of an increased amount of chlorine for its removal. In this washing operation the action of the dilute alkali solutions can be assisted by the addition of oxidizing agents, such as bleaching powder, for example, or alkali metal sulfites or wetting agents such as soap, saponine, organic solvents and the like, or by the addition of several of these agents.

As compared to bleaching processes heretofore known in the art, all varieties of cellulose may be bleached by the process of the present invention with a saving of 25-30% of active chlorine, and a product of better color and higher chemical purity is obtained. As the process may be carried out in the cold in a short time, it may be used as a continuous process without it being necessary to work with high cellulose concentrations.

## Example

Partially concentrated pulp is digested with a solution of alkali-metal or earth-alkali-metal hydroxide at temperatures between 10 and 80° C. The pulp concentration may be from 1 to 25%; the amount of alkaline react-

ing substances present may be calculated as sodium hydroxide, 0.2 to 2% by weight of the pulp. Oxidizing agents, alkali-metal sulfites, moistening agents and organic solvents 5 may be added to the liquid used for digesting. When the digestion is finished, the liquid is drawn off and the pulp is washed with water. The cellulose obtained is then treated, preferably in a closed vessel, with a measured 10 amount of aqueous solution of chlorine, containing about 70 to 90% of the total chlorine necessary for bleaching. The concentration of the cellulose may be 1-20% in this treatment. In about  $\frac{1}{4}$  to 1 hour and at a temperature of between 5 to 20° C. the chlorine present 15 is completely consumed.

When this preliminary bleaching step is finished, the treated cellulose mass is at once, or better after a thorough washing with 20 water, digested in the same manner with alkaline reacting washing liquids as described above and washed with water.

The pre-bleached cellulose mass thus obtained is partially concentrated and finished 25 by bleaching it in the known manner with neutral or alkaline reacting hypochlorite solutions.

This after-bleaching step may be accelerated, by the addition of inorganic or organic 30 salts of catalytic metals, such as copper, nickel, cobalt and the like, along with the chlorine water in the preliminary bleaching step. Because of the prevailing weakly acid reaction these salts remain in solution without 35 at first exerting any catalytic action, are intimately mixed with the fibers, and—because dissociated—are partially absorbed by the amphoteric cellulose. The catalytic compounds, thus uniformly dispersed in the fibers, are then further fixed by the alkali treatment and their catalytic action therefore 40 does not become apparent until in the bleaching step with hypochlorite.

I claim:

45 1. A method for bleaching cellulose of any kind which consists in digesting the cellulose to be bleached with diluted aqueous solutions of alkaline reacting compounds, subjecting the digested cellulose to a preliminary bleaching with an aqueous solution of gaseous chlorine in a measured amount less than the total necessary for complete bleaching, washing the pre-bleached cellulose and subjecting the washed cellulose to an after- 50 bleaching with hypochlorites.

2. A method for bleaching cellulose of any kind which consists in digesting the cellulose to be bleached with diluted aqueous solutions of alkaline reacting compounds containing an oxidizing agent, an alkali-metal sulfite, a moistening agent and an organic solvent, subjecting the digested cellulose to a preliminary bleaching with an aqueous solution of gaseous chlorine in a measured 55 amount less than the total necessary for com-

plete bleaching, washing the pre-bleached cellulose and subjecting the washed cellulose to an after-bleaching with hypochlorites.

3. A method for bleaching cellulose of any kind which consists in digesting the cellulose to be bleached with diluted aqueous solutions of alkaline reacting compounds, subjecting the digested cellulose to a preliminary bleaching with an aqueous solution of gaseous chlorine in a measured amount less than the total necessary for complete bleaching, digesting the pre-bleached cellulose with diluted aqueous solutions of alkaline reacting compounds and subjecting the digested cellulose to an after-bleaching with hypochlorites. 75

4. A method for bleaching cellulose of any kind which consists in digesting the cellulose to be bleached with diluted aqueous solutions of alkaline reacting compounds, subjecting the digested cellulose to a preliminary bleaching with an aqueous solution of gaseous chlorine in a measured amount less than the total necessary for complete bleaching, digesting the pre-bleached cellulose with diluted aqueous solutions of alkaline reacting compounds containing an oxidizing agent, an alkali-metal sulfite, a moistening agent and an organic solvent and subjecting the digested cellulose to an after-bleaching with hypochlorites. 85

5. A method for bleaching cellulose of any kind which consists in digesting the cellulose mass to be bleached with diluted aqueous solutions of alkaline reacting compounds containing an oxidizing agent, an alkali-metal sulfite, a moistening agent, and an organic solvent, washing the digested cellulose with water, subjecting the washed cellulose to a preliminary bleaching with an aqueous solution of gaseous chlorine containing about 70-90% of the chlorine necessary for complete bleaching and small amounts of salts of metals catalyzing the decomposition of hypochlorites, washing the pre-bleached cellulose with water, digesting the washed cellulose with diluted aqueous solutions of alkaline reacting compounds containing an oxidizing agent, an alkali-metal sulfite, a moistening agent and an organic solvent, washing the digested cellulose with water and subjecting the washed cellulose to an after-bleaching with solutions of hypochlorites containing the remaining amount of active chlorine necessary for bleaching. 100

In testimony whereof I affix my signature.

LADISLAV RYS.